

April 6, 1954

W. E. THOMPSON, JR., ET AL

2,674,215

THREAD BOBBIN

Filed April 3, 1952



INVENTORS

Walter E. Thompson, Jr.  
Raymond L. Hart

BY

Dennis, Edmonds, Morton, Barrows and Taylor

ATTORNEYS

## UNITED STATES PATENT OFFICE

2,674,215

## THREAD BOBBIN

Walter E. Thompson, Jr., and Raymond L. Hart,  
 Watertown, Conn., assignors to The Heminway  
 & Bartlett Mfg. Co., Watertown, Conn., a cor-  
 poration of Connecticut

Application April 3, 1952, Serial No. 280,434

8 Claims. (Cl. 112—251)

1

This invention relates to bobbins formed of continuous filament thread and has for its object the provision of improved bobbins and a method of making them. The bobbins of our invention are formed of continuous filament thread formed of filament-forming synthetic resins having an exterior coating of synthetic resinous material and are compressed while the coating material is at adhesive consistency in the direction of their axes of rotation such an amount as to effect a material reduction in thickness and to press the adjacent convolutions of thread into side-to-side adhesive contact. The improved bobbins of the invention are dense having a relatively great length of thread on a volume basis, and the convolutions of thread are so bonded together that the bobbins will not unravel but will unwind freely under the tension of the feed of the machine in which they are used.

Bobbins formed of continuous filament threads of such filament-forming synthetic resins as nylon, Orlon (polyacrylonitrile), Saran (co-polymers of vinylidene and acrylonitrile), Dacron (polyethylene glycol terephthalate), and Vinyon N (copolymer of vinyl chloride and acrylonitrile) are relatively dense and smooth and have the property of plastic memory in varying degrees. Because of the absence of projecting end-fibers, such as characterize the thread formed of staple synthetic filaments and natural fibers, the bobbins formed of continuous filament thread unravel freely and this results in delays in their use. If bobbins formed of these continuous filament threads were compressed axially, they would spring back on release of the pressure because of the smoothness, resiliency, and plastic memory of the thread.

It has been the practice heretofore in making bobbins of such continuous filament threads to wind the thread on paper cores which support the bobbins internally and then to attach paper sides to the paper core to support the bobbins on the sides. Even with this expediency, they are relatively loose and contain much less length of thread than they would have in a compressed state. The unravelling annoyance is still present and a cause of much delay and loss of thread. Moreover, the bobbin shells occupy space that is utilized with thread in the bobbins of the invention.

Bobbins having paper shells or metal bobbins for use in sewing machines have a tendency to

2

spin and release thread which causes an entanglement, thus forcing an interruption of stitching. This is particularly noticeable upon stopping and starting of the machine in normal operation. Bobbins produced by our method decrease in diameter as the thread is used resulting in a constant peripheral speed, whereas the conventional bobbins has a progressively increasing peripheral speed. Therefore, the tendency to spin is greatly reduced in the use of bobbins manufactured in accordance with our invention.

In accordance with the method of our invention, we apply to the exterior surfaces of a core strand of continuous filament synthetic threads a thin coating of a thermoplastic synthetic resinous material that softens to adhesive consistency at temperatures above 140° F., and wind the thread, preferably by standard cross-wind means to form bobbins of relatively low density and considerably larger in axial thickness than required for use in the intended machine. The synthetic resinous material of the coating is not adhesive at normal temperatures and is more compressible than the core strand. The bobbins are preferably placed over an arbor or pin to retain their internal dimensions and are compressed in the direction of their axes of rotation while at a temperature at which the resinous coating is softened to effect adhesive bonding under pressure. The bobbins are reduced in thickness at least 20%, and most advantageously to around 30%, thereby excluding most of the air, and forcing the adjacent convolutions of thread into a positive but weak side-to-side adhesive bonding. On cooling and release of pressure, the bobbins spring back but a small amount and do not unravel with normal handling. It is advantageous to form bobbins having uniformly flat sides and this is accomplished according to the invention by pressing the bobbins between dies having sloped, e. g., conically shaped surfaces, to compress the bobbins more near their centers than near their peripheries because there is a greater tendency to spring back at the center which diminishes progressively in the direction of their perimeters.

One important characteristic of the bobbins of the invention is their dimensional stability, many types of the bobbins retaining their dimensions even when exposed to high humidity at normal temperatures.

The accompanying drawing illustrates more or less diagrammatically, in sectional elevation, an arrangement of apparatus suitable for forming improved bobbins of the invention especially intended for use in sewing machines.

The apparatus illustrated in the drawings comprises a frame 1 in which a plurality of upper die blocks 2 is mounted, a movable central frame 3 on which a plurality of lower die blocks 4 is mounted, and a movable lower frame 5 on which a plurality of cylindrical pins or arbors 6 is mounted. The frame 1 is preferably fixed, while the frames 3 and 4 are reciprocable in an upward and downward direction. The frames 1, 3 and 5 are preferably heated to a sufficiently elevated temperature that the die blocks 2 and 4 and the arbors 6 are heated by conductivity to the requisite temperature for heating the bobbins.

In a preferred embodiment of the invention, the compression faces of the die blocks 2 and 4 are conically shaped, the angles  $\alpha$  varying from 1° to 5° to the end that the centers of the bobbins are compressed more than the edges.

The method of the invention will now be described with particular reference to nylon continuous filament thread, it being understood that the method may be applied with slight variations that will be apparent to those skilled in the art to the other continuous filament threads herein mentioned.

Nylon thread, twisted or braided, in varying sizes such as may be used in winding bobbins for sewing machines, net-tying machines, and lace-making machines, is coated with a synthetic resinous material in any suitable manner. The coating is preferably one that becomes thermoplastic to adhesive consistency at temperatures above 140° F. and which is not tacky at ordinary temperatures. United States Letters Patent 2,590,586 of Walter E. Thompson, Jr. and Rollin W. Taylor describes resinous coating materials and methods of application which may be utilized in carrying out a method of the invention. We prefer to use the thermoplastic coating materials described in the patent.

We shall now describe the invention in the formation of our improved bobbins from a nylon thread made of 210 denier nylon, spun 13 turns right, matched three cord, and twisted 11 turns left.

A first coating is prepared by dissolving ½ part of 66 nylon flake in a solution consisting of 2 parts of water and 8 parts of ethyl alcohol (all parts by weight).

A second coating is prepared by forming a solution comprising 110 parts of ethyl alcohol, 2½ parts polyvinyl butyral, and ½ part oleic acid (all parts by weight).

In applying the coatings, the nylon thread is first run through a bath of the first coating, then through a drying chamber as described in connection with Fig. 1 of the said patent. The second coating is applied over an emulsion roll at the time of winding the bobbin. The purpose of the second coating is to diminish the strength of the first coating and eliminate jerking in unwinding. For sewing machine bobbins we may eliminate the first coating and just use the second coating by using a higher concentration of resin than in the above coating. While the patent describes the application of coatings containing from 10% to 20% of resin on the basis of the weight of the core, such amounts of coatings are usually applied only when making bobbins for fishnets, and the like. It is to be understood that

for thread to be made into sewing machine bobbins we prefer to use considerably thinner coatings.

The coated thread when at a temperature 5 below the softening point of the coating is wound into cross-wound bobbins in any suitable manner. We prefer to wind the bobbins under an appreciable tension. When using a coating of the type just described, the bobbins are preferably placed in a chamber where they are allowed to become conditioned at a relative humidity of 40-44% at a temperature of about 80° F. The absorbed moisture aids in suppressing the plastic memory when the bobbins are heated under pressure and results in better dimensional stability. The term "plastic memory" is used herein to define that tendency of certain synthetic resinous materials to return to their original state after having been elongated. In the case of nylon thread and other thread having similar plastic memory characteristics, the suppression of plastic memory in the heating during-coating can be undone if the heating during bobbin compression is at temperatures around 250° F. in the absence of moisture. We, accordingly, prefer to heat the bobbins during compression when in a suitably moist condition.

The bobbins may be left under these moisture conditions for around 24 hours. The conditioned bobbins B are placed over the arbors 6 which are elevated to project above the die blocks 4 and then frames 3 and 5 are raised, the arbor 6 entering the central opening of die block 2. A sufficient pressure is applied to reduce the thickness 30 of the bobbins at least 20% as measured in the direction of the axis of the arbor which is the axis of rotation of the bobbin. We prefer, however, in forming nylon bobbins to reduce the thickness to from 30% to 35%. The die blocks 35 and arbors are at such temperatures that the nylon bobbins are heated to temperatures of about 260° F. and the pressure is maintained for about 60 seconds. After the compression and heating have been completed, the frame 5 is lowered to pull the arbor out of the top die block and then frame 3 is lowered slightly, at which position it is held for around 10 seconds to allow the bobbins to set. Following this, frames 3 and 5 are lowered to remove the bobbins.

50 In one preferred operation, we use die blocks in which the angle  $\alpha$  is about 2°. These die blocks give the bobbin a concave surface when under pressure, as shown by the broken lines, but when the pressure is released, the bobbins expand much more at the centers than at their peripheral edges and assume the dead flat shape shown in full lines.

A typical bobbin formed of nylon thread in the 55 operation above described had an initial thickness in its axial direction of 0.640 in. and after compression and relaxation a thickness measured in the same direction of 0.420 in. which is a reduction in thickness of 35%. Other bobbins similarly formed having an initial thickness of 0.525 in. before compression and 0.360 in. after compression were reduced in thickness 32%.

In forming bobbins of Dacron thread, we prefer to follow the same practice described in connection with the use of nylon. In forming bobbins of Orlon, however, we prefer to heat the bobbins to a temperature of around 160° F. and to hold the bobbins while under compression for about 45 seconds.

Bobbins formed of the continuous filament 70 thread herein described are usually wound over

the core of a bobbin shell which has retaining sides later pressed on to prevent unravelling. Even when so protected, the loose thread unwinds freely and can easily become entangled. The core and supporting side members occupy considerable space, as in the shuttle of a sewing machine. The improved bobbin of the invention is very dense and can be shaped to occupy the maximum space in the machine where it is intended to be used. It can be handled without unravelling. As an indication of their unravelling properties, the bobbins of the invention (with the end of thread unsecured) can be thrown against a wall as one would throw a baseball without causing unravelling. Notwithstanding this property, the bobbin can be unwound smoothly and without the necessity for undue tension, as by the tension of a sewing machine feed. Another important characteristic of the bobbins of the invention is their dimensional stability. The importance of dimensional stability is emphasized by the fact that the bobbins can be produced with such close uniformity that they do not vary more than 0.005 in. in thickness. The bobbins do not appreciably change shape. For example, nylon bobbins of the invention may be exposed to atmospheric conditions of high humidity at normal temperatures without changing shape to any appreciable extent. We attribute the characteristics of our improved bobbins to the combination of the coating and the compression. The compression removes substantially all of the air from the bobbin and brings the adjacent convolutions of thread into side-to-side bonding contact. The threads while in the bobbin appear to have some ellipticity whereby there is appreciable side-to-side attachment.

The bobbins of our invention may be of the type that are unwound from the inside or from the outside. Bobbins for use in standard sewing are usually unwound from the outside. Bobbins of the type used for making fishnets can be unwound from the inside or from the outside depending upon the kind of machine used.

In producing bobbins of nylon thread, for example, the thread may be coated with such an amount of resin coating material as to consist of from 10% to 20% of the weight of the coated thread. Such amounts of coating are suitable for forming bobbins for use in making fishnets which are knot retentive, as described in said patent. When the bobbins are to be used in standard sewing machines, satisfactory bobbins can be formed from thread having coatings consisting of from 1% to 10% of the weight of the coated thread.

The aforementioned patent is concerned primarily with water-insoluble coating resins. This invention is not limited to the use of water insoluble coating materials and utilizes water-soluble coating materials such as polyvinyl alcohol for thread to be used in sewing machines and lace-making machines.

In the foregoing description, we have emphasized the production of bobbins having flat sides because such bobbins give improved results in unwinding and contain the maximum amount of thread on the basis of diameter. However, we may use dies that will give the faces a curved or rounded surface.

We claim:

1. A bobbin of the kind described consisting of a continuous-filament thread comprised of a core of synthetic resinous material of a type

which normally has substantially plastic memory and an exterior coating of a thermoplastic resinous material which is more compressible than the core and at normal temperatures is not adhesive but which softens to adhesive consistency at temperatures above 140° F., the convolutions of said thread being in tightly compacted relationship axially of the bobbin, the adjacent sides of the convolutions of the thread, axially of the bobbin, adhering to one another with sufficient tenacity to prevent unraveling in normal handling but with insufficient tenacity to prevent unwinding when subjected to unwinding tension, the tightly-compacted condition of the thread and the adherence of the convolutions thereof to one another being the result of axial compression of the bobbin while heated to a temperature above the softening point of the resinous material of the threads, the plastic memory of the resinous material from which the thread is formed having been substantially suppressed, whereby the thread of the bobbin has relatively little plastic memory and the bobbin is dimensionally stable, the bobbin having a relatively great length of thread on the basis of its cubic content.

2. A bobbin as defined in claim 1 in which the core of the thread is formed of a synthetic resin from the group consisting of nylon, polyethylene glycol terephthalate, polyacrylonitrile, and copolymers of vinylidene chloride and acrylonitrile.

3. The method of producing a bobbin of continuous filament thread which comprises winding a bobbin of a thread of synthetic resinous material having a surface which softens at temperatures above 140° F., compressing the bobbin in the direction of its axis sufficiently to affect a substantial reduction in thickness of the bobbin

40 axially thereof and sufficiently to force the adjacent convolutions of the thread into tightly compacted relationship axially of the bobbin, subjecting the bobbin, during the compressing operation, to a temperature at least as high as the softening point of the resinous material from

45 which the thread is made, and maintaining the bobbin under pressure while subject to such latter temperature for a length of time sufficient to bring about softening of the surface of the thread and the securing of the convolutions thereof into adhesive contact axially of the bobbin, whereby the bobbin will not unravel under normal handling but will unravel freely under an unwinding tension.

55 4. The method of producing a bobbin as defined in claim 3 in which the thread is of a synthetic resinous material normally having substantial plastic memory and in which the bobbin is compressed while in a moist condition and is maintained at a sufficiently high temperature while moist for a length of time sufficient to substantially suppress the plastic memory of the resinous material thereof.

60 5. The method of producing a bobbin as defined in claim 3 in which the resinous material from which the thread is formed is a synthetic resin selected from the group consisting of nylon, polyethylene glycol terephthalate, polyacrylonitrile, and copolymers of vinylidene chloride and acrylonitrile.

65 6. The method of producing a bobbin as defined in claim 3 in which the bobbin is compressed to effect a reduction of at least 20%

7. The method of producing a bobbin as defined in claim 3 in which the bobbin is compressed between convexly-shaped dies having a slope of from 1° to 5° to compress the bobbin more in the center than at the periphery.

8. The method of producing a bobbin as defined in claim 3 in which the bobbin, after it has been reduced in thickness to the desired degree, is held under pressure for a short period to set the resinous material, the pressure to which the bobbin is subjected is relieved and the bobbin is permitted to remain before removal for a short while to relax.

## References Cited in the file of this patent

## UNITED STATES PATENTS

| Number       | Name         | Date          |
|--------------|--------------|---------------|
| 5 675,801    | Stiles       | June 4, 1901  |
| 1,135,470    | Tolman       | Apr. 13, 1915 |
| 2,001,977    | Riddell      | May 21, 1935  |
| 2,025,920    | Webber       | Dec. 31, 1935 |
| 2,448,114    | Olson et al. | Aug. 31, 1948 |
| 10 2,488,890 | Anderson     | Nov. 22, 1949 |
| 2,564,941    | Wellman      | Aug. 21, 1951 |